

## 1

3,386,916

LUBRICATING GREASE COMPOSITION  
Howard D. Moore, Chester, Norris A. Scarlett, Eastham, Wirral, and John A. Jones, Ellesmere Port, England, assignors to Shell Oil Company, New York, N.Y., a corporation of Delaware

No Drawing. Filed June 28, 1965, Ser. No. 467,728  
Claims priority, application Great Britain, July 1, 1964,

27,172/64

9 Claims. (Cl. 252—21)

### ABSTRACT OF THE DISCLOSURE

Greases useful in a non-oxidizing atmosphere comprising a lubricating oil base gelled to grease consistency with an inorganic gel coated with a surfactant of esterifying and polymerizable silicon compounds and containing 1-10% of a  $C_{10-20}$  metal soap and 1-10% of an alkali or alkaline earth metal nitrite.

This invention relates to lubricating grease compositions, particularly to grease compositions gelled with inorganic gelling agents and is particularly concerned with the improvement of the lubricating properties of such greases during operation in a non-oxidizing atmosphere.

It has been found that the lubrication of metal surfaces by conventional inorganic greases under non-oxidizing conditions, for example the lubrication of metal bearings in the helium atmosphere of an atomic reactor, results in severe pitting of the metal surfaces and a resultant premature failure of such bearings. This failure is believed to be due to an oxide layer, normally present on the bearing's surface, being abraded away. Under normal oxidizing conditions, such as is obtained when running in air, this oxide layer would be rapidly replaced, but in a non-oxidizing atmosphere this replacement does not occur and consequently there is premature bearing failure.

It has now been discovered that this difficulty can be overcome to a great extent by the incorporation in the inorganic lubricating grease of a boundary lubricant additive to minimize the abrasion of the oxide layer and an oxygen-yielding compound to react with the metal surfaces to be lubricated and renew the oxide layer.

Accordingly, a lubricating grease has been developed consisting essentially of a lubricating oil base, an inorganic gelling agent and small amounts each of (a) an alkali or alkaline earth metal salt of an aliphatic monocarboxylic acid having from 10 to 22 carbon atoms and (b) an alkali or alkaline earth metal nitrite. It is found that these lubricating grease compositions successfully reduce bearing failure under non-oxidizing conditions and that they also exhibit adequate radiation stability and high-temperature performance.

Examples of the alkali and alkaline earth metal salts of aliphatic monocarboxylic acids, hereinafter referred to as soaps, which are used as boundary lubricant additives in the grease compositions of the present invention are sodium stearate, potassium stearate, lithium stearate, lithium oleate, sodium oleate and calcium stearate. These soaps may be employed in concentrations between 1% and 10% by weight, more preferred concentrations being between 3% and 7% by weight based on the final lubricating grease composition.

Of the alkali or alkaline earth metal nitrites which

## 2

may be used as oxygen-yielding compounds for the purposes of this invention, sodium nitrite is preferred. Concentrations of nitrites are between 1% and 10% by weight, more preferred concentrations are between 2% and 7% by weight based on the final lubricating grease composition.

As has already been stated, the grease compositions of the present invention are those containing an inorganic gel material and comprise a base lubricating oil which is thickened to a grease consistency by means of such an inorganic gel material. This inorganic gel is in the form of an organo gel, that is to say one in which water has been displaced from a hydrogel of the gel material by a volatile organic liquid, such as an alcohol which, unlike the water of the hydrogel, is soluble in the base lubricating oil employed. Of the inorganic gel materials which may be used, amorphous inorganic colloids are generally suitable, silica being especially useful because of its low cost and ready availability. The organo gel should contain between 0.5% and 10% by weight of the inorganic gel material, preferably between 1% and 7% by weight. The preparation of such organo gels is disclosed in U.S. Patent 2,986,518.

It is well known that lubricating greases comprising simply a lubricating oil and an inorganic colloid tend to break down in the presence of water. One method of improving the water resistance of the grease suitable for use in connection with the present invention is to coat the particles of the organo gel material with a surface-active agent such as an esterifying or polymerizable silicon compound. Particularly suitable polymerizable or esterifying silicon compounds for this purpose are the alkyl alkoxy silanes, for example the mono-, di- or tri-methyl tri-, di- or mono-methoxy or -alkoxy silanes. It is preferred to incorporate a surface-active agent when mixing the organo gel and the hot lubricating oil, or to incorporate the surface-active agent with the organo gel and/or the oil before such mixing. Other ingredients may also be added, in this way, for example an anti-oxidant such as phenyl-alpha- or -beta-naphthylamine, preferably added to the oil before mixing. Details of the method of mixing the organo gel and the base lubricating oil are also disclosed in U.S. Patent 2,986,518.

In order to provide the lubricating grease compositions of this invention with a satisfactory resistance to water, especially under the influence of neutron radiation as is necessary when such compositions are used in atomic piles and nuclear power units, the surface-active agent (surfactant) should be present in an amount between 15% and 400% by weight of the dry inorganic gel material. In general the quantity of surface-active agent necessary will be between 50% and 250% of the weight of the dry gel material.

The base lubricating oil which is used in present grease compositions may be any of the oils of lubricating grade which are commonly used in grease manufacture. The oil may be refined—or semi-refined—paraffinic, naphthenic or asphaltic-base mineral lubricating oil or a synthetic lubricating oil having a viscosity of from about 50 to 4000 SUS at 100° F. If desired, a blend of oils of suitable viscosity may be employed instead of a single oil, by means of which a desirable viscosity within the recited range may be secured. A particularly suitable type of lubricating oil for use in high-temperature greases is residual oil, usually known as "bright stock."

The invention will now be illustrated by the following examples:

#### EXAMPLE I

A base lubricating grease composition was prepared having the formulation:

|                                                                                         | Percent wt. |
|-----------------------------------------------------------------------------------------|-------------|
| Silica                                                                                  | 5.0         |
| Dimethyldiethoxysilane (150% silica)                                                    | 7.5         |
| Phenyl-alpha-naphthylamine                                                              | 1.0         |
| High viscosity index (HVI) oil having a viscosity of 650 secs., Redwood Index at 140° F | 86.5        |

To this base lubricating grease were added 5% by weight each of sodium nitrite and sodium stearate, at ambient

5 maintained at a temperature of 200° C. by the use of electrical heaters. The flow rate of inert gas through the bearings and pressure vessel was controlled at 10 cc. per minute. Failure was indicated by increase in noise of the bearings.

Tests carried out under 300 lbs. axial load were limited to 500 hours to ensure that bearing failure was not due to normal fatigue. The normal fatigue life of a bearing at 200° C. and run at 300 lbs. axial load is somewhat over 1000 hours.

10 The inert gas used for the test, was helium and this gas was purified so as to contain less than 1 part per million of oxygen and less than 2 parts per million of water.

TABLE I

| Grease Composition       | Atmosphere | Load                                | Duration of Test in hours                       | Reason for failure                                                        |
|--------------------------|------------|-------------------------------------|-------------------------------------------------|---------------------------------------------------------------------------|
| Base grease composition. | Helium     | { 300 lbs. axial<br>5 lbs. radial } | { 209, 21, 140, 90, 168,<br>304, 70, 120, 168 } | Severe pitting of balls and to a lesser extent the inner race of bearing. |
| Example I                | Helium     | { 300 lbs. axial<br>5 lbs. radial } | 500 (4 tests)                                   | No failure.                                                               |
| Example I                | Helium     | { 300 lbs. axial<br>5 lbs. radial } | { 24 hrs. running<br>500 hrs. static }          | No failure.                                                               |
| Example II               | Helium     | { 300 lbs. axial<br>5 lbs. radial } | { 500 hrs. running<br>3 tests }                 | No failure.                                                               |
| Example III              | Helium     | { 300 lbs. axial<br>5 lbs. radial } | 500                                             | No failure.                                                               |

temperature, by mixing into the grease with a spatula on a steel plate followed by milling through a triple roll paint mill. The sodium nitrite was added as a 40% weight suspension in oil, the composition of the suspension being:

|                                                                            |                 |
|----------------------------------------------------------------------------|-----------------|
| Water                                                                      | Trace           |
| Sodium nitrite                                                             | percent wt. 40  |
| Calcium di(C <sub>14</sub> -C <sub>18</sub> alkylsalicylate)               | percent wt. 1.6 |
| A calcium sulfonate                                                        | percent wt. 6.4 |
| MVI (neutral) oil having a viscosity of 170 secs., Redwood Index at 140° F | Balance         |

The grease prior to the addition of the sodium nitrite and stearate had an IP penetration (worked) of 264 and a drop point (IP 131) of greater than 300° C. The final grease composition had an IP penetration (worked) of 45 291 and a drop point of 285° C.

#### EXAMPLE II

The base lubricating grease composition of Example I 50 containing 5% weight of sodium stearate and 2% weight of sodium nitrite. The final grease composition in accordance with the invention had an IP penetration of 258.

#### EXAMPLE III

The base lubricating grease composition of Example I 55 containing 5% weight of sodium nitrite and 5% weight of lithium stearate.

The compositions of Examples I to III and the base lubricating grease of these examples were tested by the following procedure, the results being shown in Table I. 60

#### Test procedure

The test apparatus comprised essentially a pressure vessel through which a suitable inert gas could be passed. A 0.25 horsepower motor was incorporated in said pressure vessel. The motor shaft was supported at each end of the vessel by means of ball bearings (20 mm. x 47 mm. x 14 mm. all steel) which were lubricated with about 4 grams each of the grease composition under test. The bearings were fitted with pressed steel cages and the races and balls made from SAE52100 grade steel especially heat-treated to withstand high operating temperatures. The bearings were run at 1450 r.p.m. under an applied load of either 300 lbs. axial and 5 lbs. radial (the latter being the rotor weight) or 5 lbs. radial only, and 70

35 As already stated, the grease compositions of the present invention, while successfully reducing bearing failure under non-oxidizing conditions, also retain good radiation stability. The composition of Example I and the base lubricating grease alone (known to have adequate radiation stability) were tested by the following procedure and the results are shown at Table II. It can be seen that a grease composition of this invention does show good radiation stability.

#### Radiation test procedure

40 40 cc. (4 x 10 cc.) of the grease composition under test were contained in four glass tubes (1.5 cm. x 17.5 cm.). Irradiation was in the form of beta-rays from a 4 m.e.v. linear accelerator operating at 3 m.e.v. The dose rate received by the grease was 2 or 3 megarads per minute.

TABLE II

| Grease Composition          | Radiation, Mrads | Penetration | Drop Point, °C. |
|-----------------------------|------------------|-------------|-----------------|
| Base grease composition of— | Nil              | 264         | 300             |
| Example I                   | 10               | -----       | -----           |
|                             | 30               | 289         | 300             |
|                             | 500              | 284         | 300             |
|                             | 1,000            | 291         | 285             |
| Do                          | Nil              | 277         | 272             |
|                             | 10               | 272         | 274             |
|                             | 100              | 340         | 275             |
|                             | 500              | 329         | 270             |

We claim as our invention:

1. A lubricating grease composition consisting essentially of (1) a lubricating base oil thickened to grease consistency by means of (2) an inorganic gel, (3) 1-10% by weight, basis total composition, of a salt of (a) a C<sub>10</sub>-22 aliphatic monocarboxylic acid, and (b) a metal selected from the group consisting of alkali and alkaline earth metals, and (4) 1-10% by weight, basis total composition, of a nitrite salt of a metal selected from the group consisting of alkali and alkaline earth metals.

2. A lubricating grease composition consisting essentially of (1) a lubricating base oil thickened to grease consistency by means of (2) an inorganic gel, (3) 1-10% by weight, basis total composition, of a salt of (a) a C<sub>10</sub>-22 aliphatic monocarboxylic acid, and (b) a metal selected from the group consisting of alkali and alkaline earth metals, (4) 1-10% by weight, basis total composition, of a nitrite salt of a metal selected from the group

consisting of alkali and alkaline earth metals, and (5) 50-250% by weight, basis dry inorganic gel, of a surfactant selected from the group consisting of esterifying and polymerizable silicon compounds.

3. A lubricating grease composition consisting essentially of (1) a lubricating base oil thickened to grease consistency by means of (2) an inorganic gel, (3) 3-7% by weight, basis total composition, of a salt of (a) a  $C_{10-22}$  aliphatic monocarboxyl acid, and (b) a metal selected from the group consisting of alkali and alkaline earth metals, (4) 2-7% by weight, basis total composition, of a nitrite salt of a metal selected from the group consisting of alkali and alkaline earth metals, and (5) 50-250% by weight, basis dry inorganic gel, of a surfactant selected from the group consisting of esterifying and polymerizable silicon compounds.

4. A lubricating grease composition consisting essentially of (1) a lubricating base oil thickened to grease consistency by means of (2) an inorganic gel, (3) 1-10% by weight, basis total composition, of a salt of (a) a  $C_{10-22}$  aliphatic monocarboxylic acid, and (b) a metal selected from the group consisting of alkali and alkaline earth metals, (4) 1-10% by weight, basis total composition, of sodium nitrite, and (5) 50-250% by weight, basis dry inorganic gel, of a surfactant selected from the group consisting of esterifying and polymerizable silicon compounds.

5. A lubricating grease composition consisting essentially of (1) a lubricating base oil thickened to grease consistency by means of (2) 0.5-10% by weight, basis total composition, of an inorganic gel, (3) 1-10% by weight, basis total composition, of a salt of (a) a  $C_{10-22}$  aliphatic monocarboxylic acid, and (b) a metal selected from the group consisting of alkali and alkaline earth metals, (4) 1-10% by weight, basis total composition, of a nitrite salt of a metal selected from the group consisting of alkali and alkaline earth metals, and (5) 50-250% by weight, basis dry inorganic gel, of a surfactant

selected from the group consisting of esterifying and polymerizable silicon compounds.

6. A lubricating grease composition consisting essentially of (1) a lubricating base oil thickened to grease consistency by means of (2) 1-7% by weight, basis total composition, of an inorganic gel, (3) 1-10% by weight, basis total composition, of a salt of (a) a  $C_{10-22}$  aliphatic monocarboxylic acid, and (b) a metal selected from the group consisting of alkali and alkaline earth metals, (4) 1-10% by weight, basis total composition, of a nitrite salt of a metal selected from the group consisting of alkali and alkaline earth metals, and (5) 50-250% by weight, basis dry inorganic gel, of a surfactant selected from the group consisting of esterifying and polymerizable silicon compounds.

7. The lubricating grease composition of claim 2 in which the surfactant is an alkyl alkoxy silane.

8. The lubricating grease composition of claim 7 in which the surfactant is dimethyl diethoxy silane.

9. A lubricating grease composition consisting essentially of (1) a lubricating base oil thickened to grease consistency by means of (2) 0.5-10% by weight, basis total composition, of an inorganic gel, (3) 1-10% by weight, basis total composition, of a sodium salt of a  $C_{10-22}$  aliphatic monocarboxylic acid, (4) 1-10% by weight, basis total composition, of sodium nitrite, and (5) 50-250% by weight, basis dry inorganic gel, of an alkyl alkoxy silane.

#### References Cited

##### UNITED STATES PATENTS

|           |        |                  |       |        |
|-----------|--------|------------------|-------|--------|
| 2,514,331 | 7/1950 | Morway           | ----- | 252-21 |
| 2,563,606 | 8/1951 | Kimberlin et al. | ----- | 252-28 |
| 2,648,633 | 8/1953 | Peterson et al.  | ----- | 252-28 |
| 2,986,518 | 5/1961 | Carswell et al.  | ----- | 252-28 |
| 3,227,651 | 1/1966 | Peterson         | ----- | 252-21 |

DANIEL E. WYMAN, Primary Examiner.

I. VAUGHN, Assistant Examiner.